# EUROPEAN PATENT SPECIFICATION

(11) **EP 2 274 454 B1**
(45) Date of publication and mention of the grant of the patent: **25.11.2020**
(21) Application number: 08738391.5
(22) Date of filing: 27.03.2008
(51) Int. Cl.: C22C 21/10, C22F 1/053

(54) **ALLOY COMPOSITION AND PREPARATION THEREOF**
LEGIERUNGSZUSAMMENSETZUNG UND HERSTELLUNGSVERFAHREN DAFÜR
COMPOSITION D'ALLIAGE ET SA PRÉPARATION

(30) Priority: 30.03.2007 IN DE07312007; 30.03.2007 IN DE07322007
(43) Date of publication of application: 19.01.2011
(73) Proprietor: Director General, Defence Research & Development Organisation, 110 011-New Delhi (IN)
(72) Inventor: MUKHOPADHYAY, Kumar, Ashim, Hyderabad 500 058 (IN)
(74) Representative: Regimbeau
(86) International application number: PCT/IN2008/000196
(87) International publication number: WO 2008/120237

(56) References cited:
- EP-A- 0 368 005
- EP-A- 0 377 779
- WO-A-2006/037648
- MONDAL C ET AL: "Extrusion processing of high-strength Al alloy 7055" MATERIALS AND MANUFACTURING PROCESSES, MARCEL DEKKER, NEW YORK, NY, US, vol. 22, no. 3-4, 1 March 2007 (2007-03-01), pages 424-428, XP008095331 ISSN: 1042-6914
- MONDAL C ET AL: "On the nature of T(Al2Mg3Zn3) and S(Al2CuMg) phases present in as-cast and annealed 7055 aluminum alloy" MATERIALS SCIENCE AND ENGINEERING A: STRUCTURAL MATERIALS:PROPERTIES, MICROSTRUCTURE & PROCESSING, LAUSANNE, CH, vol. 391, no. 1-2, 25 January 2005 (2005-01-25), pages 367-376, XP004698561 ISSN: 0921-5093

## Description

### TECHNICAL FIELD

The present invention provides an Aluminium-Zinc-Magnesium-Copper-Zirconium alloy extrusion and a process for preparing an Aluminium-Zinc-Magnesium-Copper-Zirconium alloy extrusion.

### BACKGROUND

Aluminum-Zinc-Magnesium-Copper-Zirconium (Al-Zn-Mg-Cu-Zr) alloys are in great demand for various strength critical applications in areas of aerospace and defence. These alloys are commonly processed in the form of sheets, plates, extrusion, forgings, etc. for various structural applications. In aerospace applications, one of the requirements is the processing of these alloys in the form of thin sheets having thickness <0.3 mm, wherein the thin sheets of Al alloys are used in combination with fibres (preferably glass fibres) to form fibre-metal laminated (FML) composites. The strength properties of the thin sheets of Al alloys used in the FML composites play an important role in deciding the tensile yield strength of the FML composites [Ad Viot and J.W. Gunnink, Fibre Metal Laminates: An Introduction, Kluwer Academic Publishers, The Netherlands, 2001]. Further, Al alloy sheets having thickness of <0.3 mm are preferred for this purpose because it improves drapability.

U.S. Pat. No. 4,477,292 and 4,832,758 discloses Aluminium-Zinc-Magnesium-Copper-Zirconium (Al-Zn-Mg-Cu-Zr) alloys as a class of very high strength aluminium alloy that can be produced via ingot metallurgical route. The increased strength properties of this category of alloys improve specific properties (in terms of strength per density and strength per Young's modulus, etc.) and, therefore, permit significant weight savings, the major emphasis in the development efforts of these alloys has been on the improvement of strength through various metallurgical processes.

U.S. Pat. Nos. 4,699,673; 4,988,394 and U.S. Patent application No.20060191609 disclose the methods of preparation of thin sheets of Al-Zn-Mg-Cu-Zr alloys having thickness up to 1.2 mm. But there is no information regarding the preparation of high strength Al-Zn-Mg-Cu-Zr sheets having thickness as low as ≤0.3 mm. The problem associated with the retention of high strength in such products is the onset of recrystallization resulting in cracking that becomes more pronounced as the sheets are progressively made thinner. However, due to the proprietary nature of the processing details of such thin sheets, there is no information on this topic in the literature.

One of the high strength Al-Zn-Mg-Cu-Zr alloy i.e. AA 7055, known in the art [Aluminium Company of America, (ALCOA) Technical Data available at www.millproducts-alcoa.com] has the composition of Al-(7.6-8.4) wt% Zn-(1.8-2.3) wt% Mg-(2-2.6) wt% Cu-(0.08-0.25) wt% Zr. The typical tensile properties of 7055 T7751 extrusions in the longitudinal direction (i.e. along the extrusion direction) are: 0.2 % proof stress = 655 MPa, UTS = 669 MPa, elongation = 11%. The T77 temper possesses strength properties that correspond to the peak aged, T6 temper, but stress corrosion cracking resistance similar to the T76 temper [ALCOA publication. Light Metal Age, October, 1991, p. 14].

US Patent Application 20040099352 discloses another high strength Al-Zn-Mg-Cu-Zr alloy comprising (in wt%) of 8.2-10%Zn, 1.95-2.5%Cu, 1.9-2.5%Mg, 0.05-0.25 % Zr. The alloy when produced by extrusion processing and peak aged gives rise to 0.2 % P.S. of 703 MPa. Another high strength, Al-Zn-Mg-Cu-Zr base alloy containing scandium, processed in the form of extrusions and heat treated to the peak aged T6 temper, have the composition of Al-8.6Zn-2.6Mg-2.4Cu-0.2 wt% Sc and an undisclosed amount of Zr [Metall. Mater. Trans. A, 30A, 1017, 1999]. The typical tensile properties of this material are: 0.2% PS = 689 MPa, UTS = 715 MPa and elongation = 11.8%. Recent work has, however, shown that Al-Zn-Mg-Cu-Zr alloys containing Zn not exceeding 8.5wt%, and Mg and Cu contents each not exceeding 2wt% are capable of attaining similar or even higher 0.2%P.S. in the peak aged temper [Minerals & Metals Review, 10, 2005, p.65]. The implication is that neither Sc addition nor Zn content in excess of 8.5 wt% is required to attain 0.2% P.S. of about 700 MPa in peak aged extrusions of these alloys. EP0377779 discloses Al-Zn-Mg-Cu-Zr extrusions with yield strengths of 593 to 620 MPa.

US Patent Application 20050056353 discloses another high strength Al-Zn-Mg-Cu-Zr-Sc alloy comprising (in wt%) of 8.5-11 %Zn, 1.8-2.4%Mg, 1.8-2.6%Cu, 0.05-0.30%Sc and at least one element from the group Zr, V and Hf not exceeding 0.5wt%. The alloy when produced by extrusion processing and peak aged gives rise to 0.2% P.S. values that range from 670 to 715 MPa. US Patent Application 20050072497 discloses yet another high strength Al-Zn-Mg-Cu-Zr alloy comprising (in wt%) of 8.3-14%Zn, 0.3-2%Cu, 0.5-4.5%Mg, 0.03-0.15%Zr and at least one element from the group Sc, Hf, La, Ce, Nd [the amount of the selected element ranging between 0.02 and 0.7wt%]. The alloy when produced by extrusion processing and peak aged showed 0.2%P.S. values ranging from 670 to 783 MPa.

A major drawback of the Sc-bearing alloys is that scandium metal is expensive. Yet another limitation of the abovementioned alloys is that scandium ores are not available in many countries including India. Recent revelations are that the fatigue properties are deteriorated by the presence of Sc in Al-Zn-Mg-Cu-Zr alloys [Scripta Materialia, Vol.52, p. 645, 2005].

There is, therefore, a tremendous scope for the further development of Aluminium-Zinc-Magnesium-Copper-Zirconium (Al-Zn-Mg-Cu-Zr) alloy having significantly high strength that have a variety of applications especially in the field of aerospace applications, wherein sheets of thickness even less than 0.30 mm are needed, and in the filed of defence applications, extrusions of various dimensions are utilized for a number of applications.

### SUMMARY

The present invention provides an Aluminium-Zinc-Magnesium-Copper-Zirconium alloy extrusion according to claim 1 and a process for preparing an Aluminium-Zinc-Magnesium-Copper-Zirconium alloy extrusion according to claim 2.

This
disclosure, not being part of the invention, provides an Aluminum-Zinc-Magnesium-Copper-Zirconium alloy of composition Al-(8-12.5)wt%Zn-(1.2-2.0)wt%Mg-(1.4-2.2)wt%Cu-(0.10-0.18)wt%Zr and method of its preparation. The disclosure, not being part of the invention, also provides a method for preparing alloy semi-products of this composition that can be further processed into significantly high strength alloy extrusions or alloy thin sheets.

One aspect of the disclosure provides an Aluminium-Zinc-Magnesium-Copper-Zirconium (Al-Zn-Mg-Cu-Zr) alloy extrusion of composition Al-(11.5-12.5)wt%Zn-(1.3-2.0)wt%Mg-(1.5-2.2) wt%Cu-(0.16-0.18)wt%Zr.

Another aspect of the disclosure, not being part of the invention, provides an Aluminium-Zinc-Magnesium-Copper-Zirconium (Al-Zn-Mg-Cu-Zr) alloy thin sheet of composition Al-(8-10)wt%Zn-(1.2-2.0)wt%Mg-(1.4-2.2) wt%Cu-(0.12-0.18)Zr.

One aspect of the present disclosure provides a process for the preparation of an Al-Zn-Mg-Cu-Zr alloy using two-step homogenization process so as to cause more effective dissolution of the solidification products, thereby enabling the alloy to retain increased solute supersaturation during subsequent thermal and mechanical processing and to obtain high strength upon aging.

Another aspect of the present disclosure provides a process of preparation of Al-Zn-Mg-Cu-Zr alloy extrusions using optimized alloy composition and extrusion processing parameters so as to enable the alloy to obtain high strength through retaining essentially unrecrystallized grain structure and imparting solutionising effect during extrusion processing.

Another aspect of the present disclosure provides a process of preparation of an Al-Zn-Mg-Cu-Zr alloy thin sheets using optimized alloy composition, homogenization treatment, rolling parameters and intermediate annealing treatments so as to enable the alloy to greatly minimize the extent of edge cracking and to obtain high strength through the retention of essentially unrecrystallized grain structure in most parts of the sheets.

Yet another aspect of the present disclosure provides a process of preparation of an Al-Zn-Mg-Cu-Zr alloy using two-step artificial aging treatment so as to enable the alloy to obtain reproducible strength properties.

Yet another aspect of the present disclosure provides a process for preparation of less than 0.30 mm thick Al-Zn-Mg-Cu-Zr alloy sheets having significantly high strength.

### BRIEF DESCRIPTION OF DRAWINGS

The above and other features, aspects, and advantages of the subject matter will become better understood with regard to the following description, appended claims, and accompanying figures where:
**FIG 1****.** Optical micrograph showing partially recrystallized grain structure in the peak aged alloy extrusions of present disclosure.
**FIG 2****.** Optical micrograph showing essentially unrecrystallized grain structure in the peak aged alloy sheets of thickness 0.28 mm of present disclosure.
**FIG 3****.** Transmission electron micrograph showing subgrain structure present in the unrecrystallized portion of the peak aged alloy extrusions of present disclosure.
**FIG 4****.** Transmission electron micrograph showing a uniform and fine distribution of strengthening η' precipitates in the peak aged alloy extrusions of present disclosure.
**FIG 5****.** Transmission electron micrograph showing a uniform and fine distribution of strengthening η' precipitates in the peak aged alloy sheets of thickness 0.28 mm of present disclosure.

### DETAILED DESCRIPTION

The present disclosure, not being part of the invention, provides an Aluminium-Zinc-Magnesium-Copper-Zirconium (Al-Zn-Mg-Cu-Zr) alloy of composition (in weight %):
Zn 8-12.5;
Mg 1.2-2.0;
Cu 1.4-2.2; and
Zr 0.10-0.18.

The present disclosure, not being part of the invention, also provides an Aluminium-Zinc-Magnesium-Copper-Zirconium (Al-Zn-Mg-Cu-Zr) alloy semi-product of composition (in weight %):
Zn 8-12.5;
Mg 1.2-2.0;
Cu 1.4-2.2; and
Zr 0.10-0.18.

One aspect of the present disclosure provides an Aluminium-Zinc-Magnesium-Copper-Zirconium (Al-Zn-Mg-Cu-Zr) alloy extrusion of composition (in weight %):
Zn 11.5-12.5;
Mg 1.3-2.0;
Cu 1.5-2.2; and
Zr 0.16-0.18.

Another aspect of the present disclosure, not being part of the invention, provides an Aluminium-Zinc-Magnesium-Copper-Zirconium (Al-Zn-Mg-Cu-Zr) alloy thin sheet of composition (in weight %):
Zn 8-10;
Mg 1.2-2.0;
Cu 1.4-2.2; and
Zr 0.12-0.18.

Further aspect of the present disclosure, not being part of the invention, provides a process for preparing Aluminium-Zinc-Magnesium-Copper-Zirconium (Al-Zn-Mg-Cu-Zr) alloy semi-products of composition Al-(8-12.5)wt%Zn-(1.2-2.0)wt%Mg-(1.4-2.2)wt%Cu-(0.10-0.18)wt%Zr. The process comprising:
a. melting a charge mixture of primary aluminium and Al-33wt%Cu master alloy;
b. adding elemental pure Zn, followed by raising the temperature of the molten charge;
c. adding Al-50wt%Mg master alloy and Mg-28wt%Zr master alloy to the molten charge followed by super heating;
d. adding grain refining nucleant pellets at a reduced temperature;
e. adding degasser pellets;
f. pouring the molten melt under argon atmosphere into a preheated metallic mould; and
g. solidifying to obtain an as-cast billet or slab of alloy.

One aspect of the present disclosure provides a process for preparing Aluminium-Zinc-Magnesium-Copper-Zirconium (Al-Zn-Mg-Cu-Zr) alloy semi-products wherein the primary aluminium has a minimum purity of 99.80 wt%.

Another aspect of the present disclosure provides a process for preparing Al-Zn-Mg-Cu-Zr alloy semi-product wherein a charge mixture comprising of 76.38 to 84.81% by weight of primary aluminium and 4.54 to 6.97% by weight of the master alloy Al-33wt%Cu is melted in an induction furnace by melting at a temperature in the range of 720 to 730°C.

Another aspect of the present disclosure, not being part of the invention, provides a process for preparing Al-Zn-Mg-Cu-Zr alloy semi-product wherein elemental pure Zn in the range of 8.15 to 12.65% by weight is added to the molten charge and the temperature of the charge is raised in the range of 735 to 745°C. Subsequently, 2.04 to 3.32% by weight of Al-50wt%Mg master alloy and 0.46 to 0.68% by weight of Mg-28wt%Zr master alloy are added and the molten alloy is superheated to a temperature in the range of 755 to 765°C for 10 to 15 minutes.

An aspect of the present disclosure provides a process for preparing Al-Zn-Mg-Cu-Zr alloy semi-product wherein the melt, at a reduced temperature in the range of 710 to720°C, is poured under argon atmosphere into a metallic mould of suitable size preheated to a temperature in the range of 145 to 155°C.

Another aspect of the present disclosure provides a process for preparing Al-Zn-Mg-Cu-Zr alloy semi-product wherein the melt is solidified to obtain an as-cast billet or slab of alloy.

The term alloy semi-product as used herein refers to as cast billets and as-cast slabs of the alloy.

One aspect of the present disclosure provides a process for preparing high strength Al-Zn-Mg-Cu-Zr alloy extrusions, said process comprising of:
a. homogenizing, scalping and extruding the as-cast billets of the alloy;
b. solution treating, quenching; stretching the alloy extrusions to obtain 1 to 1.5% permanent set; and artificial aging to obtain peak aged, high strength alloy extrusions.

Another aspect of the present disclosure provides a process for preparing high strength Al-Zn-Mg-Cu-Zr alloy extrusions of composition Al-(11.5-12.5)wt%Zn-(1.3-2.0)wt%Mg-(1.5-2.2) wt%Cu-(0.16-0.18)wt%Zr, said process comprising of:
a. melting a charge mixture of primary aluminium and Al-33wt%Cu master alloy;
b. adding elemental pure Zn, followed by raising the temperature of the molten charge;
c. adding Al-50wt%Mg master alloy and Mg-28wt%Zr master alloy to the molten charge followed by super heating;
d. adding grain refining nucleant pellets at a reduced temperature;
e. adding degasser pellets;
f. pouring the molten melt under argon atmosphere into a preheated metallic mould;
g. solidifying to obtain an as-cast billet of the alloy;
h. homogenizing, scalping and extruding the as-cast billet of the alloy;
i. solution treating, quenching, stretching the alloy extrusions to obtain 1 to 1.5% permanent set; and
j. artificial aging to obtain peak aged, high strength alloy extrusions.

Another aspect of the present disclosure provides a process for preparing high strength Al-Zn-Mg-Cu-Zr alloy extrusions wherein homogenization is carried out in two steps. The first step is carried out at a temperature in the range of 440 to 450°C for 25 to 35 h followed by a second step homogenization at a temperature in the range of 450 to 460°C for 20 to 30 h followed by cooling in air. The homogenization treatment eliminates dendritic segregation in the cast microstructure and causes more effective dissolution of the solidification products, thereby enabling the alloy to retain increased solute supersaturation during subsequent thermal and mechanical processing so as to obtain high strength upon aging.

The homogenized billets are scalped to remove the oxide layers formed on the surfaces. The scalped billets are subjected to non-destructive testing to detect casting defects.

Further aspect of the present disclosure provides a process for preparing high strength Al-Zn-Mg-Cu-Zr alloy extrusions wherein the extrusion processing of the billets is carried out at an initial billet temperature in the range of 400 to 430°C; extrusion ratio in the range of 15:1 to 25:1 and a ram speed of 2-5 mm/s.

One aspect of the present disclosure provides a process for preparing high strength Al-Zn-Mg-Cu-Zr alloy extrusions wherein solution treatment is carried out at a temperature in the range of 450 to 460°C for 1 to 2 h followed by water quenching at room temperature. The extrusions are subjected to stretching to obtain 1 to 1.5% permanent set for stress relieving purpose.

Another aspect of the present disclosure provides a process for preparing high strength Al-Zn-Mg-Cu-Zr alloy extrusions wherein the stretched alloy extrusions are subjected to two-step artificial aging at 90 to 100°C for 6 to 8 h in the first stage followed by a second stage aging in the temperature range of 120 to 125°C for 20 to 25 h. This treatment produces peak strength in the alloy extrusion in a reproducible manner.

Yet another aspect of the present disclosure provides a process for preparing high strength Al-Zn-Mg-Cu-Zr alloy extrusions using optimized extrusion processing parameters so as to enable the alloy to obtain high strength the alloy through retaining essentially unrecrystallized grain structure and imparting solutionising effect during extrusion processing.

Further aspect of the present disclosure provides a process for preparing high strength Al-Zn-Mg-Cu-Zr alloy extrusions having minimum 0.2% tensile P.S. of 750 MPa.

An aspect of the present disclosure provides a process for preparing high strength Al-Zn-Mg-Cu-Zr alloy thin sheets, said process comprising of:
a. homogenizing, scalping, hot rolling the as-cast slabs of the alloy into sheets and subsequent cold rolling of the sheets with intermediate annealing to obtain alloy sheets of required thickness; and
b. solution treating, quenching; and artificial aging to obtain peak aged, high strength alloy sheets.

Another aspect of the present disclosure, not being part of the invention, provides a process for preparing high strength Al-Zn-Mg-Cu-Zr alloy thin sheets of composition Al-(8-10)wt%Zn-(1.2-2.0)wt%Mg-(1.4-2.2) wt%Cu-(0.12-0.18)Zr, said process comprising of:
a. melting a charge mixture of primary aluminium and Al-33wt%Cu master alloy;
b. adding elemental pure Zn, followed by raising the temperature of the molten charge;
c. adding Al-50wt%Mg master alloy and Mg-28wt%Zr master alloy to the molten charge followed by super heating;
d. adding grain refining nucleant pellets at a reduced temperature;
e. adding degasser pellets;
f. pouring the molten melt under argon atmosphere into a preheated metallic mould;
g. solidifying to obtain an as-cast slab of the alloy;.
h. homogenizing, scalping, hot rolling the as-cast slabs of the alloy into sheets and subsequent cold rolling of the sheets with intermediate annealing to obtain alloy sheets of required thickness;
i. solution treating, quenching; and
j. artificial aging to obtain peak aged, high strength alloy thin sheets.

Another aspect of the present disclosure, not being part of the invention, provides a process for preparing high strength Al-Zn-Mg-Cu-Zr alloy thin sheets wherein the homogenization treatment of the as-cast slabs of the alloy is carried out at a temperature in the range of 445 to 455°C for 25 to35 h in the first step followed by a second step homogenization at a temperature in the t range of 455 to 465°C for 10 to 20 h followed by cooling in air. The homogenization treatment eliminates dendritic segregation in the cast structure. The homogenized slabs are scalped to remove the oxide layers formed on the surfaces. The scalped slabs are then subjected to the non-destructive testing to detect casting defects.

Yet another aspect of the present disclosure, not being part of the invention, provides a process for preparing high strength Al-Zn-Mg-Cu-Zr alloy thin sheets wherein the scalped slabs (having an initial thickness of 100 mm) are subjected to hot rolling at an initial billet temperature in the range of 425 to 435°C and at a linear speed of 20 m/minute to produce plates having thickness of around 22 mm. These plates are then cross-rolled using the same initial billet temperature and rolling speed to finally produce sheets having thickness of about 5 mm. During hot rolling, 4 to 8% reduction in the thickness of the billet in three passes followed by intermediate annealing at the temperature in the range of 415 to 435°C for 15 to 25 minutes. This cycle is continued till such time the targeted plate thickness of 22 mm and subsequently the sheet thickness of 5 mm is obtained. The intermediate annealing treatment is given for stress relief purposes.

Further aspect of the present disclosure, not being part of the invention, provides a process for preparing high strength Al-Zn-Mg-Cu-Zr alloy thin sheets wherein the hot rolled sheets are subjected to cold rolling at room temperature in steps such that each step involves 15 to 25% reduction in thickness in three passes and subsequent intermediate annealing at the temperature in the range of 415 to 425°C for 15 to 25 minutes followed by cooling in air. The intermediate annealing treatment is given for stress relief purpose. The process of cold rolling and subsequent intermediate annealing is repeated till the thickness of the sheet is reduced to 0.28 mm i.e. below 0.3 mm.

An aspect of the present disclosure, not being part of the invention, provides a process for preparing high strength Al-Zn-Mg-Cu-Zr alloy thin sheets wherein solution treatment of rolled sheets is carried out at a temperature range in the range of 450 to 460°C for 1 to 1.5 h followed by water quenching at room temperature.

Another aspect of the present disclosure, not being part of the invention, provides a process for preparing high strength Al-Zn-Mg-Cu-Zr alloy thin sheets wherein artificial aging is a two-step process carried out at a temperature in the range of 90 to 100°C for 6 to 8 h followed by aging at a temperature in the range of 115 to 125°C for 20 to 30 h. This treatment produces peak strength in the alloy.

One aspect of the present disclosure, not being part of the invention, is to provide a process for the preparation of high strength Al-Zn-Mg-Cu-Zr alloy in the form of sheets of thickness less than 0.3 mm having high, reproducible strength properties i.e. a minimum 0.2% tensile PS of 623 MPa in the peak aged temper.

These, as well as other aspects of the present disclosure are explained in more detail with working examples, which are intended to illustrate the working of disclosure and not intended to take restrictively to imply any limitations on the scope of present disclosure.

### EXAMPLES

### Example 1: Preparation of Al-11.8 wt% Zn-1.4 wt% Mg-1.8 wt% Cu-0.16 wt% Zr

For a 15 kg melt of the alloy of present disclosure, a mixture of 11.98 kg of primary aluminium (purity 99.80 wt% Al and the balance being 0.15 wt% Fe and 0.05 wt% Si impurities) and 0.864 kg of Al-33 wt% Cu master alloy was charged into the induction furnace. The above charge mixture was melted at 725°C. To this molten charge, 1.7 kg of pure Zn in the ingot form was added. When the charge had melted, the temperature of the molten charge was raised to 740°C and 0.364 kg of Al-50 wt% Mg master alloy and 0.092 kg of Mg-28 wt% Zr master alloy were added in the above sequence. The charge was superheated to 760°C and the whole material was held at this temperature for 10 minutes. The temperature was then reduced to 740°C and 0.03 kg of nucleant pellets were added for grain refinement purpose. After 5 minutes, 0.04 kg of degasser pellets were added for degassing purpose. The molten alloy, at a temperature of 720°C, was then poured under argon atmosphere into a preheated (to the temperature of 150°C) metallic mould of suitable size.

The melt was solidified and the ingot was cleared of the portions having casting defects. A cylindrical as-cast billet of 95 mm diameter and 250 mm height was obtained. The billet was subjected to two-step homogenization treatment comprising of 24 h at 445°C followed by 24 h at 455°C followed by cooling in air. The billet was scalped, machined to produce 74 mm diameter cylindrical billets and cut into two halves along the length. Cylindrical billets of 74 mm diameter and 125 mm height were ready for subsequent extrusion processing. Billets were extruded at an initial billet temperature of 420°C, extrusion ram speed of 3 mm/sec and extrusion ratio of 20:1. The extrusions were solution treated at 460°C for 1.5 h, quenched in water at ambient temperature and peak aged using a two-step aging treatment involving 8 h at 100°C in the first step followed by aging at 120°C for 24 h in the second step. This heat treatment produced peak strength in the alloy. These peak aged extrusions were then utilized for evaluation of the tensile properties (see Table 1).

### Example 2: Preparation of Al-12.1 wt% Zn-1.5 wt% Mg-1.8 wt% Cu-0.16 wt% Zr

For a 15 kg melt of the alloy of present disclosure, a mixture of 11.85 kg of primary aluminium (minimum purity 99.80 wt% Al and the balance being 0.15 wt% Fe and 0.05 wt% Si impurities) and 0.86 kg of Al-33 wt% Cu master alloy was charged into the induction furnace. The above charge mixture was melted at 725°C. To this molten charge, 1.84 kg of pure Zn in the ingot form was added. When the charge had melted, the temperature of the molten charge was raised to 740°C and 0.36 kg of Al-50 wt% Mg master alloy and 0.09 kg of Mg-28 wt% Zr master alloy are added in the above sequence. The charge was superheated to 760°C and the whole material was held at this temperature for 10 minutes. The temperature was then reduced to 740°C and 0.03 kg of nucleant pellets were added for grain refinement purpose. After 5 minutes, 0.04 kg of degasser pellets were added for degassing purpose. The molten alloy, at a temperature of 720°C, was then poured under argon atmosphere into a preheated (to the temperature of 150°C) metallic mould of suitable size.

When the melt was solidified, the ingot was cleared of the portions having casting defects. A cylindrical as-cast billet of 95 mm diameter and 250 mm height was obtained. The billet was subjected to two-step homogenization treatment comprising of 24 h at 445°C followed by 24 h at 455°C followed by cooling in air. The billet was scalped, machined to produce 74 mm diameter cylindrical billets and cut into two halves along the length. Cylindrical billets of 74 mm diameter and 125 mm height were ready for subsequent extrusion processing. Billets were extruded at an initial billet temperature of 420°C, extrusion ram speed of 3 mm/sec and extrusion ratio of 20:1. The extrusions were solution treated at 460°C for 1.5 h, quenched in water at ambient temperature and peak aged using a two-step aging treatment involving 8 h at 100°C in the first step followed by aging at 120°C for 24 h in the second step. This heat treatment produced peak strength in the alloy. These peak aged extrusions were then utilized for evaluation of the tensile properties (see Table 2).

### Example 3 (reference): Preparation of Al-8.3wt%Zn-1.9wtMg-1.7wt%Cu-0.18wt%Zr

For a 50 kg melt of the present disclosure, a mixture of 41.154 kg of primary aluminium (purity 99.85 wt% Al and the balance being a maximum of 0.09 wt% Fe and 0.06 wt% Si impurities) and 2.72 kg of Al-33 wt% Cu master alloy was charged into the induction furnace. The above charge mixture was melted at 725°C. To this molten charge, 4.225 kg of pure Zn in the ingot form was added. When the charge had melted, the temperature of the molten charge was raised to 740°C and 1.562 kg of Al-50 wt% Mg master alloy and 0.339 kg of Mg-28 wt% Zr master alloy were added in the above sequence. The charge was superheated to 760°C and the whole material was held at this temperature for 10 minutes. The temperature was then reduced to 740°C and 0.10 kg of nucleant pellets were added for grain refinement purpose. After 5 minutes, 0.25 kg of degasser pellets were added for degassing purpose. The molten alloy at the temperature of 720°C, was then poured under argon atmosphere into a preheated (to the temperature of 150°C) metallic mould of suitable size.

When the melt was solidified, the ingot was cleared of the portions having casting defects. A rectangular as-cast billet of 340 mm (length) × 300 mm (width) × 100 mm (thickness) was then obtained. The billet was subjected to the homogenization annealing in two steps annealing at 450°C for 25 h in the first step and annealing at 460°C for 15 h in the second step followed by cooling in air. The homogenized billet was scalped in order to remove the oxidized layers on the surfaces of the billet. The billet was subjected to hot rolling. Hot rolling was carried out at an initial billet temperature of 425°C and at a linear speed of 20 m per minute. Following 6% reduction in thickness of the billet in three passes, and subsequent intermediate annealing at 430°C for 20 minutes for stress relief purposes, the same hot rolling cycle was continued till such time the targeted plate thickness of 22 mm was achieved and subsequent cross rolling was carried out to obtain the sheet thickness of 5 mm. The hot rolled sheets were then subjected to cold rolling. Following 20% reduction in thickness in three passes and subsequent intermediate annealing at 420°C for 15 minutes for stress relief, the sheets were subjected to the same cycle till such time the thickness of 0.28 mm i.e. the targeted thickness of below 0.30 mm was achieved. The sheets were then subjected to solution treatment at 460°C for 1 h followed by water quenching at room temperature. The sheets were then subjected to artificial aging at 100°C for 8 h followed by artificial aging at 120°C for 24 h. This heat treatment produced peak strength in the alloy. These peak aged materials were then utilized for evaluation of the tensile properties (see Table 3).

### Example 4 (reference): Preparation of Al-9.5wt%Zn-1.6wtMg-2.0wt%Cu-0.17wt%Zr

For a 50 kg melt of the present disclosure, a mixture of 40.536 kg of primary aluminium (purity 99.85 wt% Al and the balance being a maximum of 0.09 wt% Fe and 0.06 wt% Si impurities) and 3.03 kg of AI-33 wt% Cu master alloy was charged into the induction furnace. The above charge mixture was melted at around 725°C. To this molten charge, 4.825 kg of pure Zn in the ingot form was added. When the charge had melted, the temperature of the molten charge was raised to 740°C and 1.288 kg of Al-50 wt% Mg master alloy and 0.321 kg of Mg-28 wt% Zr master alloy were added in the above sequence. The charge was superheated to 760°C and the whole material was held at this temperature for 10 minutes. The temperature was then reduced to 740°C and 0.10 kg of nucleant pellets was added for grain refinement purpose. After 5 minutes, 0.25 kg of degasser pellets was added for degassing purpose. The molten alloy at the temperature of 720°C was then poured under argon atmosphere into a preheated (to the temperature of 150°C) metallic mould of suitable size.

When the melt was solidified, the ingot was cleared of the portions having casting defects. A rectangular as-cast billet of 340 mm (length) × 300 mm (width) × 100 mm (thickness) was then obtained. The billet was subjected to the homogenization annealing in two steps annealing at 450°C for 25 h in the first step and annealing at 460°C for 15 h in the second step followed by cooling in air. The homogenized billet was scalped in order to remove the oxidized layers on the surfaces of the billet. The billet was subjected to hot rolling. Hot rolling was carried out at an initial billet temperature of 425°C and at a linear speed of 20 m per minute. Following 6% reduction in thickness of the billet in three passes, and subsequent intermediate annealing at 430°C for 20 minutes for stress relief purposes, the same hot rolling cycle was continued till such time the targeted plate thickness of 22 mm was achieved and subsequent cross rolling was carried out to obtain the sheet thickness of 5 mm. The hot rolled sheets were then subjected to cold rolling. Following 20% reduction in thickness in three passes and subsequent intermediate annealing at 420°C for 15 minutes for stress relief, the sheets were subjected to the same cycle till such time the thickness of 0.28 mm i.e. the targeted thickness of below 0.30 mm was achieved. The sheets were then subjected to solution treatment at 460°C for 1 h followed by water quenching at room temperature. The sheets were then subjected to artificial aging at 100°C for 8 h followed by artificial aging at 120°C for 24 h. This heat treatment produced peak strength in the alloy. These peak aged materials were then utilized for evaluation of the tensile properties (See Table 4).

### Example 5: Evaluation of the Alloy

The tensile properties of the alloys of examples 1-4 of present disclosure were examined using tensile tests carried out at ambient temperature on tensile specimens (25 mm gauge length). The alloys of example 1 and 2 were tested on round bar tensile specimens (25 mm gauge length) while alloy of example 3 and 4 were tested on flat tensile specimens. Tables 1 to 4 represent the tensile test results for examples 1 to 4, respectively.

The most noticeable feature of these results is the significantly high 0.2% P.S. values i.e. a minimum 0.2% P.S. of 755 MPa for the high strength alloys of example 1 and 2 and a minimum 0.2% P.S. of 623 MPa for the high strength thin sheets of alloys of example 3 and 4. **Figure 1** shows the partially recrystallized grain structure in the peak aged alloy extrusions of present disclosure. The obtained data of 0.2% P.S. values is consistent with the retention of subgrain structure (**Figure 3**) in the predominantly unrecrystallized grain structure in the peak aged alloy extrusions and essentially unrecrystallized grain structure in the peak aged sheets of thickness 0.28 mm (**Figure 2**) of present disclosure. It also characterizes the presence of a uniform and fine distribution of strengthening ή precipitates in the peak aged alloy extrusions (**Figure 4**) and alloy thin sheets (**Figure 5**).

It may be noted that the alloys of present disclosure was prepared using ≤99.85 wt% purity primary Al. Therefore, it is understood that the ductility (i.e. % elongation) of the alloys when prepared using higher purity e.g. 99.9 wt% Al would be considerably higher.

**Table 1. Tensile Properties of Peak Aged Alloy Extrusions of Example 1 of Present Disclosure**

| Serial No. | 0.2% PS (MPa) | UTS (MPa) | % Elongation |
|---|---|---|---|
| 1 | 755 | 765 | 6.1 |
| 2 | 768 | 782 | 5.4 |
| 3 | 758 | 772 | 5.8 |
| 4 | 762 | 779 | 5.7 |
| 5 | 769 | 779 | 6.2 |

**Table 2. Tensile Properties of Peak Aged Alloy Extrusions of Example 2 of Present Disclosure**

| Serial No. | 0.2% PS (MPa) | UTS (MPa) | % Elongation |
|---|---|---|---|
| 1 | 760 | 764 | 6.8 |
| 2 | 783 | 789 | 5.4 |
| 3 | 766 | 778 | 5.3 |
| 4 | 780 | 789 | 6.5 |
| 5 | 776 | 781 | 6.0 |

**Table 3. Tensile Properties of 0.28 mm Thick Peak Aged Alloy Sheets of Example 3 of present disclosure**

| Serial No. | 0.2% PS (MPa) | UTS (MPa) | % Elongation |
|---|---|---|---|
| 1 | 656 | 723 | 4.8 |
| 2 | 657 | 708 | 4.7 |
| 3 | 658 | 715 | 6.0 |
| 4 | 661 | 709 | 4.5 |
| 5 | 655 | 710 | 4.5 |
| 6 | 656 | 717 | 7.2 |
| 7 | 655 | 710 | 6.4 |
| 8 | 650 | 707 | 6.5 |
| 9 | 623 | 681 | 7.3 |
| 10 | 651 | 702 | 6.3 |

**Table 4. Tensile Properties of 0.28 mm Thick, Peak Aged Alloy Sheets of Example 4 of Present disclosure**

| Serial No. | 0.2% PS (MPa) | UTS (MPa) | % Elongation |
|---|---|---|---|
| 1 | 692 | 755 | 5.3 |
| 2 | 685 | 751 | 4.9 |
| 3 | 689 | 760 | 5.1 |
| 4 | 703 | 778 | 8.3 |
| 5 | 727 | 799 | 9.0 |
| 6 | 705 | 770 | 7.9 |
| 7 | 712 | 772 | 6.5 |
| 8 | 691 | 758 | 6.4 |
| 9 | 690 | 760 | 5.0 |
| 10 | 685 | 746 | 4.8 |

## Claims

1. An Aluminium-Zinc-Magnesium-Copper-Zirconium (AI-Zn-Mg-Cu-Zr) alloy extrusion of composition in weight%:
Zn 11.5-12.5;
Mg 1.3-2.0;
Cu 1.5-2.2; and
Zr 0.16- 0.18, and balance being Aluminium,
wherein said alloy extrusion having high strength and essentially retaining unrecrystallized grain structure and imparting solutionising effect during extrusion processing.

2. A process for preparing Aluminium-Zinc-Magnesium-Copper-Zirconium (Al-Zn-Mg-Cu-Zr) alloy extrusion of composition claimed in claim 1, said process comprising:
a. melting a charge mixture of primary aluminium and Al-33%wt%Cu master alloy;
b. adding elemental pure Zn, followed by raising the temperature of the molten charge;
c. adding Al-50%wtMg master alloy and Mg-28wt%Zr master alloy to the molten charge followed by super heating;
d. grain refinement by adding nucleant pellets at a reduced temperature;
e. degassing by adding degasser pellets;
f. pouring the molten melt under argon atmosphere into a preheated metallic mould;
g. solidifying to obtain an as-cast billet of alloy,
h. subjecting the billet to homogenization treatment comprising of 25 -35 h at 440- 450°C followed by 20-30 h at 450- 460 °C followed by cooling in air;
i. scalping and machining;
j. extruding the machined billet imparting solutionising effect during extrusion processing
k. solution treating, quenching in water; and
l. two-step aging treatment for 6 - 8 h at 90 - 100°C in the first step followed by aging at 120 - 125°C for 20 - 25 h in the second step to obtain high strength alloy essentially retaining unrecrystallized grain structure.

3. The process as claimed in claim 2 wherein the extrusion processing is carried out at initial billet temperatures in the range of 400-430°C, extrusion ratio in the range of 15:1 to 25:1 and a ram speed of 2-5 mm/s.

4. The process as claimed in claim 2 wherein solution treatment is carried out in the temperature range of 450-460°C for 1-2 h followed by water quenching at room temperature.

## Patentansprüche

1. Aluminium-Zink-Magnesium-Kupfer-Zirconium-Legierungsextrusion (Al-Zn-Mg-Cu-Zr) mit der folgenden Zusammensetzung in Gewichts-%:
Zn 11,5 bis 12,5;
Mg 1,3 bis 2,0;
Cu 1,5 bis 2,2; und
Zr 0,16 bis 0,18 und wobei der Rest Aluminium ist,
wobei die Legierungsextrusion eine hohe Festigkeit aufweist und im Wesentlichen eine nicht rekristallisierte Kornstruktur bewahrt und während der Extrusionsverarbeitung Lösungswirkung verleiht.

2. Verfahren zur Herstellung von Aluminium-Zink-Magnesium-Kupfer-Zirconium-Legierungsextrusion (Al-Zn-Mg-Cu-Zr) mit der Zusammensetzung nach Anspruch 1, wobei das Verfahren umfasst:
a. Schmelzen einer Beschickungsmischung aus Primäraluminium und Al-33-Gew.-%-Cu-Vorlegierung;
b. Hinzugeben von reinem Elementar-Zn, gefolgt vom Erhöhen der Temperatur der geschmolzenen Beschickung;
c. Hinzugeben von Al-50-Gew.-%-Mg-Vorlegierung und Mg-28-Gew.-%-Zr-Vorlegierung zu der geschmolzenen Beschickung, gefolgt von Überhitzung;
d. Kornfeinen durch Hinzugeben von Nukleationspellets bei einer verringerten Temperatur;
e. Entgasen durch Hinzugeben von Entgasungspellets;
f. Gießen der geschmolzenen Schmelze unter Argonatmosphäre in eine vorgeheizte metallische Form;
g. Erstarren zum Erhalten eines wie gegossenen Knüppels aus Legierung;
h. Unterziehen des Knüppels einer Homogenisierungsbehandlung, die von 25 bis 35 Std. bei 440 bis 450°C, gefolgt von 20 bis 30 Std. bei 450 bis 460°C, gefolgt von Kühlung in Luft umfasst;
i. Grobsieben und Bearbeiten;
j. Extrudieren des bearbeiteten Knüppels, wobei der während der Extrusionsverarbeitung Lösungswirkung verliehen wird,
k. Lösungsbehandlung, Abschrecken in Wasser, und
l. Auslagerungsbehandlung in zwei Stufen während 6 bis 8 Std. bei 90 bis 100°C im ersten Schritt, gefolgt von Auslagern bei 120 bis 125°C während 20 bis 25 Std. im zweiten Schritt, um eine Legierung mit hoher Festigkeit zu erhalten, die eine im Wesentlichen nicht rekristallisierte Kornstruktur bewahrt.

3. Verfahren nach Anspruch 2, wobei die Extrusionsverarbeitung bei Ausgangsknüppeltemperaturen im Bereich von 400 bis 430°C, mit einem Formänderungsverhältnis im Bereich von 15:1 bis 25:1 und einer Kolbengeschwindigkeit von 2 bis 5 mm/s durchgeführt wird.

4. Verfahren nach Anspruch 2, wobei die Lösungsbehandlung im Temperaturbereich von 450 bis 460°C während 1 bis 2 Std., gefolgt von Abschrecken in Wasser bei Raumtemperatur durchgeführt wird.

## Revendications

1. Produit d'extrusion d'alliage d'aluminium-zinc-magnésium-cuivre-zirconium (Al-Zn-Mg-Cu-Zr) ayant la composition suivante, en % en poids :
Zn 11,5 à 12,5 ;
Mg 1,3 à 2,0 ;
Cu 1,5 à 2,2 ; et
Zr 0,16 à 0,18, le reste étant de l'aluminium,
dans lequel ledit produit d'extrusion d'alliage a une résistance élevée et conserve essentiellement une structure de grains non recristallisés et confère un effet solubilisant durant le traitement d'extrusion.

2. Procédé pour préparer un produit d'extrusion d'alliage d'aluminium-zinc-magnésium-cuivre-zirconium (Al-Zn-Mg-Cu-Zr) ayant la composition selon la revendication 1, ledit procédé comprenant :
a. la fusion d'un mélange de charge d'aluminium primaire et d'alliage maître d'Al à 33 % en poids de Cu ;
b. l'addition de Zn élémentaire pur, suivie de l'élévation de la température de la charge fondue ;
c. l'addition d'un alliage maître d'Al à 50 % en poids de Mg et d'un alliage maître de Mg à 28 % en poids de Zr à la charge fondue, suivie d'un sur-chauffage ;
d. l'affinage de grains par addition de pastilles d'agent de nucléation à une température réduite ;
e. le dégazage par addition de pastilles de dégazeur ;
f. le versement de la masse fondue, dans une atmosphère d'argon, dans un moule métallique préchauffé ;
g. la solidification pour que soit obtenue une billette d'alliage telle que coulée ;
h. la soumission de la billette à un traitement d'homogénéisation comprenant 25 à 35 heures à 440-450 °C suivies de 20 à 30 heures à 450-460 °C suivies d'un refroidissement dans l'air ;
i. l'écroûtage et l'usinage ;
j. l'extrusion de la billette usinée, ce qui confère un effet de solubilisation durant le traitement d'extrusion ;
k. le traitement en solution, la trempe dans de l'eau ; et
l. le traitement de vieillissement en deux étapes pendant 6 à 8 heures à 90-100 °C dans la première étape suivies d'un vieillissement à 120-125 °C pendant 20 à 25 heures dans la deuxième étape pour que soit obtenu un alliage haute résistance conservant essentiellement une structure de grains non recristallisés.

3. Procédé selon la revendication 2, dans lequel le traitement d'extrusion est mis en œuvre à des températures initiales de billette situées dans la plage allant de 400 à 430 °C, un rapport d'extrusion situé dans la plage allant de 15/1 à 25/1, et une vitesse de pilon de 2 à 5 mm/s.

4. Procédé selon la revendication 2, dans lequel le traitement en solution est mis en œuvre à une température située dans la plage allant de 450 à 460 °C pendant 1 à 2 heures suivies d'une trempe dans de l'eau à la température ambiante.
